

## 1

3,098,694

## CONTINUOUS TREATMENT OF WOOL TO SHRINK-

## PROOF AND SENSITIZE THE SAME

Malcolm J. Reider, Shillington, Pa., assignor to Drew Chemical Corporation, a corporation of Delaware  
No Drawing. Filed July 11, 1960, Ser. No. 41,760  
14 Claims. (Cl. 8—128)

The present invention is directed to the treatment of wool, usually in the form of fabric but not limited thereto, and fabrics containing wool, hair, fur or other keratinous fibers, for the purpose of stabilizing the same against shrinkages and distortion.

In the weaving operations stresses are set up in the fabric which are released on wetting or other treatment thereof resulting in relaxation shrinkage. Also as the fabric ages as by washing, wearing, etc., additional milling or felting takes place. These phenomena are disadvantageous as they interfere with the fabrication thereof into garments, for example, and they may cause undesirable shrinkages in the garments, causing them to get out of shape. Methods have been proposed to prevent such relaxation and milling or felting shrinkage but they had the defect of being batch processes which interfered with the conduct of other treatments normally conducted on such fabrics.

The present invention is intended and adapted to overcome the deficiencies of the prior art, it being among the objects of the invention to provide a substantially continuous method of treating wool fabrics to stabilize the same against relaxation shrinkage, milling and felting.

It is also among the objects of the invention to provide a process which will sensitize the fabric and stabilize it without interfering with normal treatments.

It is further among the objects of the invention to provide a process which is operable in a much shorter time than prior processes of this type, thereby rendering the process more economical.

It is still further among the objects of the invention to devise a process in which the shrinkproofing materials are not critical in the proportions thereof used in the operation.

In practicing the invention the wool fabric is passed through a bath containing a strong acid, such as sulfuric in order to deposit on or in the wool, either in combination or physically, a substantially amount of the acid. The content of acid is important and it is present on the wool in amounts of about 2.5% to 15%, the preferred range being 5% to 12% on the weight of the wool. In the next step the fabric is passed through a mixture in solution of bromate and halide in which the relative proportions of the salts may be varied widely with good results. A wetting agent inert to halogen is used to facilitate the treatment, such agents being, for example, condensation products of ethylene oxide and octyl- or nonyl-phenols. The excess acid is neutralized, as with sodium bicarbonate, while leaving the wool still on the acid side. Then the fabric is treated with an aqueous solution of an alkali metal sulfite or bisulfite in sufficient amount to neutralize the free bromine plus an amount sufficient to reduce the disulfide linkages in the wool, which is then dried. The wool is then in a sensitized condition.

The thus sensitized fabric may be dried at a temperature below about 175°—180° F. to retain its sensitiveness. A garment may be made therefrom and permanent creases or pleats may be formed therein by subjecting the garment to temperatures above about 175°—180° F., as in the standard steam pressing machine to set the fabric. If the drying is conducted at these higher temperatures in the piece, while the fabric is held flat and smooth, then the fabric will be smooth, creaseless and not sub-

## 2

ject to further shrinkage or felting; and garments made therefrom will retain their shapes through many cleanings or washings. If the drying is at or above 175°—180° F. only about two minutes treatment are required so that the total fabric treatment may be continuous. At temperatures of, say, 140°—150° F. as much as 10 to 15 minutes are required for the drying operation.

The following is a specific example of the operation of the invention:

10 The fabric to be treated is passed through a solution of 14% sulfuric acid in water, plus a small amount of wet-out material such as the condensation product of ethylene oxide and octyl phenol. The temperature of the sulfuric acid solution is maintained between 100° and 120° F. to assist in rapid wetting and combination of the wool with the sulfuric acid present.

15 The fabric is then squeezed in a pad machine to a pickup of 75%. With a pickup of 75% of a 14% solution of sulfuric acid, the net result being that the fabric contains 10% of its weight of sulfuric acid. In the event that a squeeze is used that leaves a different amount of liquor on the fabric, the initial concentration of sulfuric acid should be varied so that the fabric on leaving the pad actually contains 10% of its weight of sulfuric acid.

20 The fabric is then passed through a solution consisting of 2% potassium bromate and 7% potassium bromide. This is actual solution percentage. The temperature of this solution is maintained at 120° to 140° F. and the acidified fabric on passing through this bath is again squeezed to approximately 75% pickup. The fabric thus treated is then held for a period of two minutes to permit the reaction between the freed bromine and the wool to take place. This time delay can be achieved by "skying" 25 the goods or holding it in a "J box" for this length of time.

30 The fabric is next passed through a washer or other suitable unit containing a solution of sodium bicarbonate and sodium sulfite sufficient to neutralize the excess acid 35 and the free halogen. A 3% solution of sodium bicarbonate containing 1/2% of sodium sulfite is sufficient for this purpose. The temperature of this solution is about 120° to 140° F. Instead of the potassium bromate-potassium bromide stated above, 2% potassium bromate and 12% sodium chloride may be used to effect the same shrinkproofing reaction.

35 After passing the treated fabric through a clear water solution to wash out soluble salts, and squeezing, it is now ready for finishing in the usual manner and is now shrinkproofed. It is most expeditious to perform this treatment 40 immediately after an acid fulling or milling operation has been completed. Milling or fulling of any type will not be effective on the goods after shrinkproofing has been applied.

45 The stabilization of the fabric involves the reduction of the disulfide linkages in the wool molecules by sodium bisulfite solution to produce a sensitized fabric. That is, a fabric that upon being subjected to steaming and/or heating in a fixed position will tend to remain in that fixed 50 position. As an example: the steam pressing of sensitized fabric in a steam press to create a crease as in trousers or pleated skirts that will be permanent and withstand laundering in the ordinary home-type washer.

55 In the present process, immediately after the application of the bromate and bromide solution, the fabric is treated with sodium bicarbonate to neutralize the traces of remaining acids, and in addition, a sufficient amount of sodium sulfite is added to neutralize any free halogen that might be present and react with the wool to reduce disulfide linkages and to perform the sensitizing reaction 60 as well.

65 For example, the fabric is passed into a 2% sodium bi-

carbonate solution, or an amount of bicarbonate sufficient to maintain a pH of 5.0 on the fabric. To this same sodium bicarbonate solution is added 3% of sodium sulfite. It is necessary that the amount of bicarbonate added to this amount of sulfite is such that the fabric will when passing through the sensitizing bath, and after being squeezed, have a pH of  $5.0 \pm 0.5$ . The temperature of this solution is held at about 140° F. and the goods remain in the bath for a few seconds. The excess solution is then squeezed from the fabric and the fabric is held for about 5 minutes to complete the sensitizing reaction. At the end of 5 minutes the fabric is washed in water no hotter than about 125° F. and squeezed. At this point the fabric is sensitized and ready for further processing by one of two methods.

*Method No. 1 for Utilizing Sensitized Fabric*

If the fabric is dried at a temperature below 180° F. with plenty of moving air to facilitate the rapid drying, it will be in a condition wherein it can accept a crease by pressing on a steam press for approximately 30 seconds using a damp press-cloth and steam of 60 pounds pressure. After pressing and allowing to air dry for a period of 24 hours, this crease will be permanent and will withstand repeated laundering in a home-type washer. At no time prior to the pressing of the pleats or creases must the fabric, that has been sensitized, be permitted to reach a temperature in excess of 180° F., especially in the presence of steam. If this is allowed to happen the cloth will lose its sensitivity and be unable to undergo a permanent creasing or pleating operation.

*Method No. 2 for Utilizing Sensitized Fabric*

The sensitized wet fabric may be subjected to a stabilizing treatment by passing it while still damp over a series of drying cans or large mangles until it is ironed dry with no added tension being placed upon the fabric.

Instead of drying cans, the goods can be fed while still damp onto a semi-decator, a crab, tenter-frame or other similar device designed to steam the goods in a fixed flat controlled position. Fabric that has been treated in this way is then dried in a conventional dryer at usual temperatures using over-feed so as to introduce no tension, and finished in the usual manner.

Another method of producing the stabilized fabric is to dry the goods at a temperature below 180° F., again with an abundance of moving air, and then subjecting the fabric to the normal shearing, cropping, napping, lustering, polishing and/or other dry finishing processes, being careful to avoid any process that would introduce heat in the order of 175°-180° F. The fabric in a sensitized condition, while being given this preliminary finishing treatment, should not be subjected to a steaming operation. After the preliminary finish has been applied, the fabric can then be wound onto a decating device and subjected to the usual decating process. Or in the case of developing a polished or high luster nap, a heated polishing roll or iron may be used to simultaneously polish and set the fabric.

In the claims the use of the term "wool" is intended to include all keratinous fibers amenable to the process.

What is claimed is:

- 5 1. A continuous method of treating wool to shrink-proof and sensitize the same which comprises—
  - (1) passing said wool through a bath of an aqueous solution of an acid and depositing on said wool about 2.5% to 15% of said acid based on the weight of said wool,
  - (2) then passing said wool through an aqueous solution of an alkali metal bromate and an alkali metal salt of an acid radical taken from the class consisting of bromide and chloride,
  - (3) thereafter neutralizing excess of acid while leaving said wool on the acid side, and
  - (4) subsequently passing said wool through an aqueous solution of a substance taken from the class consisting of alkali metal sulfite and bisulfite
  - (5) and at a temperature not over about 175° F. to sensitize said wool.
- 10 2. A method according to claim 1 wherein the sensitized wool is dried at temperatures below about 175° F.
- 15 3. A method according to claim 1 wherein the sensitized wool is dried at temperatures above about 175° F. to stabilize said wool in a current of steam.
- 20 4. A method according to claim 1 wherein the amount of acid carried by said wool is about 5% to 12%.
- 25 5. A method according to claim 1 wherein the temperature of said acid treatment is about 100° to 120° F.
- 30 6. A method according to claim 1 wherein the wool picks up about 75% of a 2% bromate solution.
- 35 7. A method according to claim 1 characterized in that the temperature of bromination and of sulfiting is about 120-140° F.
- 40 8. A method according to claim 1 wherein the neutralization is to a pH of about 4.5 to 5.5.
- 45 9. A method according to claim 1 wherein the ratio of bromate to halide is from 1-4 of bromate to 8-1 of halide, respectively.
- 50 10. A method according to claim 1 wherein a wetting agent resistant to halogenation is employed.
- 55 11. A method according to claim 1 wherein an excess of said sulfite is present in sufficient amount to reduce sulfide linkages to sensitize the wool.
12. A method according to claim 1 wherein the amount of said sulfite is sufficient to neutralize free bromine but insufficient to sensitize said wool.
13. A method according to claim 1 wherein the sensitized wool is dried at temperatures above about 175° F. to stabilize said wool.
14. A method according to claim 13 wherein the wool in the form of fabric is under stress during said stabilization.

**References Cited in the file of this patent**

**UNITED STATES PATENTS**

- |           |              |               |
|-----------|--------------|---------------|
| 2,714,051 | Barnes ----- | July 26, 1955 |
| 2,739,034 | Fell -----   | Mar. 20, 1956 |
| 2,923,596 | Levin -----  | Feb. 2, 1960  |